

Patented Sept. 25, 1923.

1,468,937

# UNITED STATES PATENT OFFICE.

PERCY A. E. ARMSTRONG, OF LOUDONVILLE, NEW YORK, ASSIGNOR TO LUDLUM STEEL COMPANY, OF WATERVLIET, NEW YORK, A CORPORATION OF NEW YORK.

## ALLOY STEEL AND ARTICLES MADE THEREFROM.

No Drawing. Continuation of applications filed April 10, 1919. Serial Nos. 289,152 and 289,153. This application filed November 11, 1922. Serial No. 600,434.

To all whom it may concern:

Be it known that I, Percy A. E. Armstrong, a subject of the King of Great Britain, and a resident of Loudonville, county of Albany, State of New York, have invented certain new and useful Improvements in Alloy Steel and Articles Made Therefrom, of which the following is a specification.

- 10 My invention relates to an improved alloy steel and articles made therefrom. This improved alloy steel may be used for a variety of purposes, including cylinders and plungers for high pressure extrusion work, 15 shafts and gears for automobiles and the like, shear blades, punches and dies, broaches, rivet sets, and various other purposes requiring a steel of unusually high strength. It is particularly well adapted 20 for impact tools, such as hand and pneumatic chisels, punches, beading tools, smiths' tools and the like.

My improved alloy steel has a number of characteristic qualities adapting it for uses, 25 such as referred to and particularly for impact tools. Tools made therefrom can be hardened to take and retain a sharp cutting or penetrating edge or point. It is homogeneous and tough, and cutting edges or 30 points do not break or chip off. When a tool made therefrom is hardened so that it cannot be filed, it can be bent without breaking, by the application of sufficient force.

My improved steel has a considerable 35 quenching range for hardening, running all the way from about 1500° to 2100° F. The higher it is heated within this range before quenching, the harder it gets. By reason of having so considerable a range for quenching, it is easy for the ordinary smith to obtain a proper quenching temperature with the facilities at his disposal, and without 40 the use of pyrometers or other devices for making accurate temperature determinations.

An alloy steel in accordance with the present invention may be of analysis about as follows, the percentages being by weight:

|                   |      |    |       |
|-------------------|------|----|-------|
| 50 Carbon -----   | .30% | to | .60%  |
| Manganese -----   | .20% | to | .60%  |
| Silicon -----     | .20% | to | .60%  |
| Chromium -----    | .75% | to | 1.75% |
| Tungsten -----    | 1%   | to | 2.5%  |
| 55 Vanadium ----- | .10% | to | .85%  |

The rest iron with small proportions of impurities, such as sulphur, phosphorus, copper and the like. A small proportion of nickel, say up to about .5%, may be present without harmful effect.

60 The following is a typical example of alloy steel made in accordance with my invention, and same is given for illustration and for affording an understanding of my invention only and without limitation of 65 the invention, as variations may be made within the range stated without departing from my invention:

|                  |         |    |
|------------------|---------|----|
| Carbon -----     | .35 %   | 70 |
| Manganese -----  | .50 %   |    |
| Silicon -----    | .30 %   |    |
| Chromium -----   | 1.25 %  |    |
| Tungsten -----   | 2.10 %  |    |
| Vanadium -----   | .30 %   | 75 |
| Iron -----       | 94.84 % |    |
| Sulphur -----    | .015%   |    |
| Phosphorus ----- | .015%   |    |
| Copper -----     | .08 %   |    |

80 Cold chisels and punches, for example, made from my improved alloy steel, of substantially the composition just given, may be hardened by quenching down from about 1500° to 2100° F. and, when so hardened, 85 have a very high degree of cutting or penetrating power, and can, nevertheless, be bent right up to the cutting edge or point without breaking. Punches made therefrom and driven cold through carbon steel have their points bent to the side if ground somewhat off center. Chipping tools made therefrom, particularly if thin, will bend after continued use and may then be turned over and used, in turned over position, until they 90 bend reversely, and this may be done repeatedly without breaking.

95 The following specific example is given for illustration and for affording an understanding of an embodiment of my invention 100 only and without limitation of the invention as variations may be made within the ranges stated without departing from my invention.

Several cold chisels were made of alloy steel of composition given above as a typical example. These chisels were heat treated all alike by heating to about 1700° F. and quenching in water. One of these chisels was tested against the best chisels which could be obtained in the market.

Several such chisels, made from the best chisel steel which was available on the market, were tested on a piece of railroad rail and of the lot but one penetrated the rail to the extent of as much as half an inch before breaking down.

One of the chisels made in accordance with my invention and of the composition above stated, was then inserted in this half 10 inch cut and driven entirely through the cold metal by long continued blows of heavy sledge hammers, and even after this treatment the head of the chisel was battered only slightly and the tool was in good condition for further use. Then a second chisel 15 made from the same bar, was supported by its ends and bent considerably by sledge hammer blows without breaking.

I have repeatedly seen punches made in 20 accordance with my invention driven clear through blocks of carbon steel three or four inches thick, so that the punch came out on the opposite side, and at times, when the punch point happened to be ground slightly 25 out of center, it would be deflected or bent, so that, on coming out, the point was curved or bent to one side, looking very much like a shoemaker's curved awl punched through a piece of leather. Chisels of this steel, 30 when used in a pneumatic tool, for example, for chipping defective spots out of bars of tool steel during its manufacture will bend to one side after long continued use, particularly if the chisel is comparatively thin. 35 When this occurs, it is only necessary to turn the chisel over, so that its opposite side is directed toward the surface or object being chipped and the chipping or other work can be proceeded with, using the same 40 chisel, only in turned over position, and substantially without interruption of the work, and this can be done repeatedly.

An electric crucible furnace can be used to good advantage in making the alloy steel 45 of the present invention, but the use of other furnaces or apparatus may be resorted to, if desired, so long as substantially the desired components and proportions are retained.

50 While I have referred to certain uses for which alloy steel in accordance with my invention is well adapted, it is to be understood that such uses are referred to only in order to give an understanding of some of 55 the characteristic qualities of my improved alloy steel and that the invention is not limited to such uses, but that the same may be made use of wherever steel, having the characteristic qualities described, may be 60 utilized to advantage.

The present application comprises the subject matter of my copending applications Serial No. 289,152 and Serial No. 289,153, both filed on April 10, 1919, and is a continuation of said prior applications.

I claim:

1. An alloy steel consisting substantially of carbon about .30 to .60%, manganese about .20 to .60%, silicon about .20 to .60%, chromium about .75% to 1.75%, tungsten about 1.0% to 2.5%, and vanadium about .10 to .85%, and the principal part of the remainder iron. 70

2. An alloy steel consisting substantially of carbon, manganese and silicon under .6% 75 and over .2% each, chromium about .75% to 1.75%, tungsten about 1.0% to 2.5%, vanadium about .10% to .85%, and the principal part of the remainder iron.

3. An alloy steel for impact penetration 80 tools having a quenching range from about 1500° to 2100° F., and capable of being bent without breaking when quenched down from such temperatures and of analysis substantially as follows: carbon about .30 to .60%, manganese about .20 to .60%, silicon about .20 to .60%, chromium about .75 to 1.75%, tungsten about 1.0 to 2.5%, vanadium about .10 to .85%, and the principal part of the remainder iron. 85

4. An alloy steel having composition substantially as follows: carbon about .35%, manganese about .50%, silicon about .30%, chromium about 1.25%, tungsten about 2.10%, vanadium about .30%, and the principal part of the remainder iron. 95

5. As a new article of manufacture, an impact tool of the class described and containing carbon about .30-.60%, manganese about .20-.60%, tungsten about 1.0-2.5%, vanadium about .10-.85%, chromium about .75-1.75%, and the principal part of the remainder iron. 100

6. As a new article of manufacture, an impact tool of the class described and containing carbon about .35%, manganese about .50%, silicon about .30%, chromium about 1.25%, tungsten about 2.10%, vanadium about .35% and the principal part of the remainder iron. 105

7. An impact tool for operating on metal made from alloy steel containing carbon about .20-.60%, chromium about .75-1.75%, tungsten about 1-2.5%, vanadium about .10-.85%, and the principal part of the remainder iron, cooled rapidly from a temperature in the neighborhood of 1700° F., having a high penetrative power and adapted to be bent without breaking. 115

8. An impact tool for operating on metal formed of alloy steel of analysis about as follows: Carbon, manganese and silicon each .20-.60%, chromium .75-1.75%, tungsten 1-2.5%, vanadium .10-.85%, and the principal part of the remainder iron, quenched from a temperature somewhat over the critical point and under 2100° F., having a high penetrative power and adapted to be bent to a material extent without breaking. 120

9. A sharpened impact tool for operating 125

on metal, such as a chisel, punch or the like, formed of alloy steel of analysis about as follows: carbon, silicon and manganese each .20-.60%, chromium .75-1.75%, tungsten 1-2.5%, vanadium .10-.85%, and the remainder iron with traces of impurities, cooled rapidly from a temperature somewhat above the critical point and under 2100° F., having a high penetrative power and adapted to be bent to a material extent without breaking.

In testimony whereof, I have signed my name hereto.

PERCY A. E. ARMSTRONG.